

W. S. NUTTER.

MOHAIR FABRIC.

APPLICATION FILED NOV. 26, 1913. RENEWED JAN. 11, 1915.

1,131,259.

Patented Mar. 9, 1915.

Fig. 1.



Fig. 2.



Fig. 3.



Witnesses.

J. Morill Fuller  
William E. Gagen

Inventor.  
William S Nutter,  
by Edward Smith & Tennant,  
Atty's.

# UNITED STATES PATENT OFFICE.

WILLIAM S. NUTTER, OF SANFORD, MAINE, ASSIGNOR TO GOODALL WORSTED COMPANY, OF SANFORD, MAINE, A CORPORATION OF MAINE.

## MOHAIR FABRIC.

1,131,259.

Specification of Letters Patent. Patented Mar. 9, 1915.

Application filed November 26, 1913, Serial No. 803,310. Renewed January 11, 1915. Serial No. 1,714.

To all whom it may concern:

Be it known that I, WILLIAM S. NUTTER, a citizen of the United States, residing at Sanford, county of York, State of Maine, have invented an Improvement in Mohair Fabric, of which the following description, in connection with the accompanying drawing, is a specification, like characters on the drawing representing like parts.

10 This invention relates to mohair fabric and has for its objects to provide a fabric of this type which resembles linen in appearance, which is cheaper to manufacture, and is stronger and more durable than the 15 ordinary mohair fabric, and which is peculiarly adapted for use in the manufacture of summer clothing.

A mohair fabric is one made wholly or partly from a yarn spun from the fleece of 20 the Angora goat. The Angora fleece contains fibers of two different characters, that is, a white fiber with comparatively little life which will not take a dye readily, and another fiber with considerable life which 25 will readily take the dye. The first-named white fiber that will not readily take the dye is known to the trade as "kemp" and will be hereinafter referred to as kemp. The white fibers comprising the so-called 30 kemp are usually coarse fibers somewhat larger than the other fibers which will readily take the dye.

In preparing yarn from the Angora fleece, it has heretofore been customary to subject 35 the fleece to the combing process to an extent sufficient not only to take out the noil, but also to remove the so-called kemp while leaving in the top from which the yarn is spun the fibers which will readily take a 40 dye. In thus continuing the combing operation to a point sufficient to remove the kemp, a considerable part of the other fibers which will readily take a dye are removed, so that a considerable per cent. of the original 45 material of the Angora fleece is removed during the process of removing the kemp. This necessarily adds to the cost of mohair yarn.

In making my improved cloth, I employ 50 an unbleached, undyed mohair yarn made from tops having the above-mentioned kemp therein. In other words, the Angora fleece from which the mohair yarn in my improved cloth is made is simply combed sufficiently to remove the noil and the top thus

produced with the kemp therein is drawn and spun into yarn of the desired size. This yarn can be produced much more cheaply than the ordinary mohair yarn because of the fact that it is not necessary to comb the 60 tops to the extent required to remove the kemp therefrom.

In making up my new fabric I propose to use the mohair yarn thus produced for the weft and to employ a specially-prepared 65 warp thread which cooperates with this mohair weft yarn to produce goods of an even texture. The presence of the kemp in the weft yarn of the fabric gives the yarn a somewhat uneven appearance, partly because of the fact that these kemp fibers are whiter than the other fibers of the yarn, and partly because of the fact that many of them are larger and coarser and thus tend to stand out more or less prominently. If 70 an undyed, unbleached yarn of this nature is woven into a cloth having a plain warp thread, the appearance of the cloth will be more or less streaky due to the uneven streaky character of the weft yarn produced 75 by the presence of the kemp therein. In order to break up this streaky appearance in the cloth and to produce a cloth having an even texture, I propose to employ a variegated warp thread showing different colors, 80 such for instance as would be produced by twisting together two strands which are formed of different colors. For making a tan-colored fabric I find best results are secured by employing a warp thread having 85 a white and a colored strand twisted together, the colored strand being approximately twice the size of the white strand but the particular colors of the two strands may be varied according to the character of 90 the cloth to be produced. When two strands of this nature are twisted together to the right extent, a warp thread is produced which when used in conjunction with a mohair weft yarn or thread, such as above described, will produce a fabric having uniform color, the colored and white warp threads operating to break up any streaky 95 appearance which would be produced by the particular weft yarn above described.

In order to give a better understanding of the invention I would refer to the accompanying drawings.

Figure 1 is a view of a piece of cloth made in accordance with my invention; Fig. 2 is 110

an enlarged and somewhat exaggerated view of the weft yarn; Fig. 3 is a similar view of the warp thread which may be used in the fabric.

5 Referring to Fig. 2 which represents the weft yarn 10, the white fibers of the yarn constituting the kemp are shown at 3 and the other fibers at 4. An unbleached, undyed mohair yarn made from tops including both of these fibers presents a somewhat streaky or uneven appearance illustrated in Fig. 2. As above described, the warp thread 7 which is used in weaving the cloth is one showing different colors, the object of 15 using a warp of this nature being to break up and counteract the streaky appearance due to the presence of the kemp fibers 3 in the weft yarn 10. In the preferred embodiment of my invention I secure a warp thread 20 of this character by twisting together two strands 5 and 6 of different color, the strand 5 being a white or light-colored strand and the strand 6 being a strand having a darker color. Where the fabric being produced is a 25 tan-colored fabric, the strand 5 will preferably be a white strand and the strand 6 will be a tan-colored strand, but the particular color of the strands 6 may be varied somewhat, depending on the color of the cloth to be 30 produced.

I find best results are secured by making the colored strand 6 approximately twice the size of the white strand 5. The fabric 8 is made by interweaving these warp and 35 weft threads in ordinary manner. A fabric of this nature can be produced much more cheaply than an ordinary mohair fabric due to the less cost of producing the mohair yarn. Further, such a fabric has all the 40 appearance of a linen fabric and is exceptionally well adapted for use in making hot-weather suits, such as linen is commonly used for.

The fabric can be washed without danger 45 of shrinking or change of color because it is unbleached and undyed, and as the full strength of the fiber is maintained the cloth

is stronger and more durable than the ordinary mohair cloth.

It will be obvious, of course, that the style 50 or pattern of the cloth embodying my invention may be varied by introducing at proper intervals colored threads to produce a stripe or a check effect. An important feature of the invention is the use in the cloth of a 55 variegated thread showing different colors to break up and eliminate the streaky appearance of the cloth due to the presence of the white kemp fibers in the mohair yarn.

Having fully described my invention what 60 I claim as new and desire to secure by Letters Patent is:

1. A fabric comprising warp threads and weft threads, one of said threads containing the fibers of the Angora fleece that will readily take a dye and also the so-called kemp fibers of the fleece that will not readily take a dye, and the other thread being a variegated thread showing different colors throughout its length to break up the streaky 70 appearance of the fabric due to the presence of the kemp fibers in the first named thread.

2. A fabric comprising a weft formed from mohair yarn spun from tops containing both the fibers of the Angora fleece 75 which will readily take a dye and the fibers constituting the kemp, and a two-ply warp formed of a white strand and a colored strand twisted together.

3. A fabric comprising a weft formed 80 from mohair yarn spun from tops having both the fibers of the Angora fleece that will readily take a dye and the fibers constituting the kemp, and a two-ply warp formed of a white strand and a colored strand twisted 85 together, said colored strand being approximately twice the size of the white strand.

In testimony whereof, I have signed my name to this specification, in the presence of two subscribing witnesses.

WILLIAM S. NUTTER.

Witnesses:

WILLIAM BATCHELDER,  
CLYDE L. REED.